

Sept. 2, 1969

S. F. GALASSO

3,464,785

PROCESS FOR PRODUCING ORDERED COMPLEX PEROVSKITE-TYPE

CRYSTALS WITH HIGH DIELECTRIC CONSTANTS

Filed Dec. 14, 1965

2 Sheets-Sheet 1

FIG. 1

LOG RESISTIVITY VS TEMPERATURE FOR  
A Ba(Mg<sub>0.33</sub> Ta<sub>0.67</sub>)O<sub>3</sub> SINGLE CRYSTAL



Sept. 2, 1969

S. F. GALASSO

3,464,785

PROCESS FOR PRODUCING ORDERED COMPLEX PEROVSKITE-TYPE  
CRYSTALS WITH HIGH DIELECTRIC CONSTANTS

Filed Dec. 14, 1965

2 Sheets-Sheet 2

FIG. 2

DIELECTRIC CONSTANT VS TEMPERATURE FOR  
A Ba(Mg<sub>0.33</sub>Ta<sub>0.67</sub>)<sub>2</sub> SINGLE CRYSTAL



# United States Patent Office

3,464,785

Patented Sept. 2, 1969

1

3,464,785

## PROCESS FOR PRODUCING ORDERED COMPLEX PEROVSKITE-TYPE CRYSTALS WITH HIGH DIELECTRIC CONSTANTS

Salvatore F. Galasso, Manchester, Conn., assignor to 5 United Aircraft Corporation, East Hartford, Conn., a corporation of Delaware

Filed Dec. 14, 1965, Ser. No. 513,735

Int. Cl. C01g 35/00; B01d 9/00; H01b 3/02

U.S. Cl. 23—51

3 Claims

### ABSTRACT OF THE DISCLOSURE

Perovskite-type single crystals of the formula



wherein A is barium or strontium and B' is magnesium, calcium, zinc, nickel or cobalt are prepared by mixing powders of a compound yielding the oxide of A with  $Ta_2O_5$  and the B' metal oxide and then mixing the powders with a flux of the formula  $AF_2$ , wherein A is as defined above. The resulting mixture is heated to a temperature above the melting point of the flux and after holding for at least 0.5 hours is gradually cooled to effect crystal formation.

This invention relates in general to materials characterized by high, temperature-stable dielectric constants. It contemplates the production of ordered complex perovskite-type crystals with dielectric constants which are relatively unaffected thermally up to temperatures as high as 800° C.

In the electronics industry the more common capacitor compounds which are dielectrically temperature-stable, exhibit dielectric constants on the order of approximately 10. Those materials, including the ferroelectrics such as barium titanate, which possess dielectric constants several orders of magnitude larger than the usual capacitor compounds, are known to be temperature sensitive. A need exists in the industry for capacitor insulators displaying both high dielectric constants and reasonable thermal stability, particularly in the higher temperature ranges.

Accordingly, it is a fundamental object of this invention to provide materials exhibiting high electrical resistivity properties over a wide temperature range.

A further object of this invention is to provide ordered complex perovskite-type crystals characterized by high dielectric constants which are substantially independent of their environment up to temperatures of 800° C.

An additional object is to provide methods of producing crystals of high electrical resistivity from compounds identified by the formula  $A(B'_{0.33}B''_{0.67})O_3$ , particularly those characterized by the formula  $A(B'_{0.33}Ta_{0.67})O_3$ .

These and other objects and advantages of this invention will be set forth in the following description or will be evident therefrom or from practice of the invention.

FIGURE 1 is a graph of log resistivity versus temperature for a representative  $Ba(Mg_{0.33}Ta_{0.67})O_3$  single crystal.

FIGURE 2 is a graph of dielectric constant versus temperature for a  $Ba(Mg_{0.33}Ta_{0.67})O_3$  single crystal.

The perovskite structure is recognized in the art as that adopted by many  $ABO_3$ -type compounds in which large A ions and oxygen ions form close-packed layers with small B ions in the octahedral holes between the oxygen ions. Investigations have been made of a large number of new compounds of the general formula  $A(B'_x B''_{y})O_3$ , where B' and B'' are two different elements in the octahedrally coordinated cation position of the perovskite structure. Experiments have confirmed that many com-

2

pounds identified by the formula  $A(B'_{0.33}B''_{0.67})O_3$  form in an ordered perovskite structure. Inorganic Chemistry, 2, 482 (1963). Complete ordering has been found in those materials of the  $A(B'_{0.33}Ta_{0.67})O_3$  type, which can best be described as a hexagonal unit cell containing three close-packed  $BaO_3$  layers with the B' and Ta ions arranged in the octahedral holes.

Compounds were prepared with the divalent B' ions selected to obtain compounds with differences ranging from 0.01 to 0.52 in the radii of the B' and Ta ions, and where A was a barium or strontium ion. The structural data for the  $A(B'_{0.33}Ta_{0.67})O_3$  compounds prepared, including cell sizes, ionic radii of the divalent B' ions, and the difference in ionic radii of the B ions is presented in Table I.

TABLE I  
[Structure data for  $A(B'_{0.33}Ta_{0.67})O_3$  compounds]

| Compound                    | Cell size, A. <sup>d</sup> | Ionic radii of B' ion, A. <sup>e</sup> | Diff. in ionic radii of B ions, A. <sup>e</sup> |
|-----------------------------|----------------------------|----------------------------------------|-------------------------------------------------|
| $Ba(Mg_{0.33}Ta_{0.67})O_3$ | {<br>a=5.782<br>c=7.067    | {                                      | 0.67                                            |
| $Ba(Ni_{0.33}Ta_{0.67})O_3$ | {<br>a=51758<br>c=7.052    | {                                      | .69                                             |
| $Ba(Co_{0.33}Ta_{0.67})O_3$ | {<br>a=5.776<br>c=7.082    | {                                      | .05                                             |
| $Ba(Zn_{0.33}Ta_{0.67})O_3$ | {<br>a=5.782<br>c=7.097    | {                                      | .74                                             |
| $Ba(Mn_{0.33}Ta_{0.67})O_3$ | {<br>a=5.819<br>c=7.127    | {                                      | .80                                             |
| $Ba(Cd_{0.33}Ta_{0.67})O_3$ | {<br>a=4.167<br>c=5.952    | {                                      | .29                                             |
| $Ba(Ca_{0.33}Ta_{0.67})O_3$ | {<br>a=5.895<br>c=7.284    | {                                      | .31                                             |
| $Ba(Pb_{0.33}Ta_{0.67})O_3$ | {<br>a=4.250<br>c=5.652    | {                                      | .52                                             |
| $Sr(Mg_{0.33}Ta_{0.67})O_3$ | {<br>a=5.652<br>c=6.951    | {                                      | .01                                             |
| $Sr(Ni_{0.33}Ta_{0.67})O_3$ | {<br>a=5.607<br>c=6.923    | {                                      | .01                                             |
| $Sr(Co_{0.33}Ta_{0.67})O_3$ | {<br>a=5.630<br>c=6.937    | {                                      | .05                                             |
| $Sr(Zn_{0.33}Ta_{0.67})O_3$ | {<br>a=5.664<br>c=6.951    | {                                      | .06                                             |
| $Sr(Ca_{0.33}Ta_{0.67})O_3$ | {<br>a=5.764<br>c=7.096    | {                                      | .31                                             |

Single crystals of the general type  $A(B'_{0.33}Ta_{0.67})O_3$  were prepared and were found to possess unique electrical properties. As representative of these unique properties, reference is made to FIGURES 1 and 2 in the drawings. Single crystals of the compound,



for example, where A is a barium ion and B' is a magnesium ion, exhibit an electrical resistivity greater than  $10^{13}$  ohm/cm. at 100° C., maintaining a resistivity of more than  $10^5$  ohm/cm. up to 800° C. Further, as best seen in FIGURE 2, this crystal is characterized by a dielectric constant of approximately 500 which is relatively independent of temperature over the above-mentioned temperature range. This was completely unexpected inasmuch as similar electrical resistivity measurements in powder compacts of substantially the same composition did not display equivalent electrical properties. While the exact reasons for the superior electrical properties of the crystal are not known, a comparison of the respective X-ray patterns associated with the various crystals showed that the perovskite pseudo-cells were less distorted in the crystal. It is postulated that the presence of a small amount of fluoride ion in the crystals produced, the fluoride ion being present in the flux in which the crystals were grown, is a contributing factor.

The preferred technique for growing crystals of the  $A(B'_{0.33}Ta_{0.67})O_3$  type is as follows, the production of the  $Ba(Mg_{0.33}Ta_{0.67})O_3$  crystals being specified for the sake of simplicity:

Reagent grade  $BaCO_3$ ,  $Ta_2O_5$  and  $MgO$  were dry-mixed in the approximate proportions to obtain stoichiometric compositions with the amount of fluoride flux as indi-

cated in Table II. The fluoride flux,  $\text{BaF}_2$ , was selected in the preparation of the  $\text{Ba}(\text{B}'_{0.33}\text{Ta}_{0.67})\text{O}_3$  type crystals, instead of the more commonly used KF,  $\text{PbO}$  or  $\text{PbO-PbF}_2$  fluxes, in order to minimize the amount of cation impurities introduced into the crystals. While  $\text{BaCO}_3$  was used in the preparation of the crystals discussed, other compounds, such as  $\text{BaNO}_3$ , from which barium oxide may be derived, are useable in the process. Similarly, although  $\text{MgO}$  was used in the preparation of the  $\text{Ba}(\text{Mg}_{0.33}\text{Ta}_{0.67})\text{O}_3$  crystals, in other instances the divalent metal oxide,  $\text{B}'\text{O}$ , was used, corresponding to the  $\text{B}'$  ion which was to be included in the compound prepared. The carbonates, nitrates and other sources of  $\text{B}'\text{O}$  are also useable in the preparation of these compounds.

The mixtures were placed in 50 ml. covered platinum crucibles and heated to a temperature approximately 100° C. above the melting point of the flux. Soaking at temperature was effected for periods ranging from 0.5 to 8.5 hours, depending on the composition of the mixture. Upon completion of soaking, the crucibles and contained samples were gradually cooled over a temperature range of approximately 400° C. and the resulting crystals were mechanically extracted from the flux. The specific soaking temperatures, soaking times, sample weights, flux rates and cooling rates are given in Table II. While the tabled conditions represent the best of numerous experiments designed to increase the size of the crystals, it will be understood that these conditions are representative only. Appropriate variations in these parameters are well within the knowledge of those skilled in the art.

TABLE II  
Conditions for growing  $\text{Ba}(\text{B}'_{0.33}\text{Ta}_{0.67})\text{O}_3$  type crystals

| Compound                                                      | Max. temp., °C. | Soaking time, hr. | Sample wt., g. | Flux wt., g. | Cooling rate, °C./hr. |
|---------------------------------------------------------------|-----------------|-------------------|----------------|--------------|-----------------------|
| $\text{Ba}(\text{Ca}_{0.33}\text{Ta}_{0.67})\text{O}_3$ ----- | 1,365           | 1                 | 6.4            | 24.0         | 13                    |
| $\text{Ba}(\text{Mg}_{0.33}\text{Ta}_{0.67})\text{O}_3$ ----- | 1,400           | 8.5               | 6.4            | 43.0         | 10                    |
| $\text{Ba}(\text{Zn}_{0.33}\text{Ta}_{0.67})\text{O}_3$ ----- | 1,380           | 2                 | 11.2           | 65.0         | 10                    |
| $\text{Ba}(\text{Ni}_{0.33}\text{Ta}_{0.67})\text{O}_3$ ----- | 1,360           | 0.5               | 6.3            | 18.0         | 40                    |

Crystals prepared in accordance with the above-described techniques were nearly cubic in shape and varied in color from yellow to green. Selected crystals from each batch were analyzed using X-ray diffraction techniques and photographs were taken using a 57.3 mm. radius Philips X-ray camera and high intensity copper  $\text{K}\alpha$  radiation, and the presence of ordering and cell sizes were determined.

For the purpose of investigating the electrical resistance and capacitance properties of the crystals, gold electrodes were placed on two faces of the largest crystals and the specimens were mounted between opposing platinum electrodes in a resistance-heated furnace. The D.C. resistance of each crystal was then measured as a function of temperature by monitoring the current while a constant voltage was applied across the faces. Capacitance measurements were obtained with a Boonton Model 74C-58 capacitance bridge using a frequency of 100 kc. In the electrical measurements made, no hysteresis effect was uncovered.

The high resistivities and large dielectric constants of these crystals, which were seen to be essentially invariant with temperature, make them attractive as dielectrics in electronic microcircuitry which may be subjected to temperature variations and temperature extremes.

While the present invention has been described in connection with several preferred embodiments and condi-

tions, no limitation is intended thereby except as defined in the following claims.

What is claimed is:

1. The method of preparing ordered complex perovskite-type crystals of the general formula



having a high temperature-stable dielectric constant comprising:

10 mixing powders consisting of a compound from which  $\text{BaO}$  may be obtained,  $\text{Ta}_2\text{O}_5$ , and

a divalent metal oxide identified by the formula  $\text{B}'\text{O}$ , where  $\text{B}'$  is selected from the group consisting of magnesium, calcium, zinc, nickel and cobalt in the proportions to obtain a stoichiometric composition according to the formula  $\text{Ba}(\text{B}'_{0.33}\text{Ta}_{0.67})\text{O}_3$ ;

mixing the powders with a fluoride flux identified by the formula  $\text{BaF}_2$ ;

heating the mixture to a soaking temperature above the melting point of the flux;

holding the mixture at the soaking temperature for at least 0.5 hour;

gradually cooling the mixture to effect crystal formation;

and extracting the crystals from the flux.

2. The method of preparing ordered complex perovskite-type crystals identified by the formula



having a high temperature-stable dielectric constant comprising:

mixing powders consisting of

$\text{BaCO}_3$ ,  $\text{Ta}_2\text{O}_5$ , and  $\text{MgO}$  in the proportions to obtain a stoichiometric composition according to the formula  $\text{Ba}(\text{Mg}_{0.33}\text{Ta}_{0.67})\text{O}_3$ ;

mixing the powders with a  $\text{BaF}_2$  flux;

heating the mixture in a covered platinum container to a soaking temperature above the melting point of the flux;

holding the mixture at the soaking temperature for at least 0.5 hours;

gradually cooling the mixture to effect crystal formation;

and extracting the crystals from the flux.

3. The method of claim 2 in which the mixture is heated to a soaking temperature approximately 100° C. above the melting point of the flux, and held at the soaking temperature for approximately 8.5 hours, and the mixture is gradually cooled over a temperature range of approximately 400° C. to effect crystal formation.

#### References Cited

#### UNITED STATES PATENTS

2,812,234 11/1957 Robinson ----- 23—51  
3,340,074 9/1967 Herzog ----- 23—51 X

#### OTHER REFERENCES

Galasso et al., "Journal of the American Chemical Soc.", vol. 81, 1959, pp. 820—823.

Galasso et al., "Inorganic Chemistry," vol. 2, 1963, pp. 482—484.

65 HERBERT T. CARTER, Primary Examiner

U.S. CL. X.R.

252—63.5